

## UNITED STATES PATENT OFFICE

HANS SCHUHMANN, OF BERLIN-CHARLOTTENBURG, AND FRIEDRICH STREUBER, OF BERLIN-TEGEL, GERMANY, ASSIGNEES TO GENERAL ELECTRIC COMPANY, A CORPORATION OF NEW YORK

## ARTIFICIAL SILK

No Drawing. Application filed December 7, 1928, Serial No. 324,574, and in Germany January 11, 1928.

The present invention relates to the manufacture of artificial silk.

We have discovered that synthetic resins of the polyhydric alcohol-polybasic acid type,

5 also known as alkyd resins, have the combination of properties required for textile fibres, and also that such resins may be fashioned, as by extrusion under high pressure, into the form of fine fibres. Such fibres are highly  
10 elastic, strong and resistant to the action of chemical reagents and solvents.

In carrying out our invention a synthetic resin is extruded through a fine orifice at a temperature of about 150 to 200° C. The resin 15 in preferably should be carried to the intermediate stage of condensation commonly known as B-stage, but should not be carried to the final completely condensed C-stage, and may be associated with various plasticizing or 20 softening agents, such as triphenyl or tricresyl phosphate, in accordance with known practice. Although our invention contemplates the use of an alkyd resin consisting mainly of glycerol and phthalic anhydride, 25 other polyhydric alcohols and other polybasic acids may be used in combination, for example, succinic acid may be used to wholly or partly replace phthalic anhydride, and glycols may be used to replace the glycerine, 30 either wholly or in part.

The resin from which the fibres are fashioned may be initially colored with suitable dyes thereby dispensing with a separate dyeing operation. The fine filament resulting 35 from the extrusion process is brought to a stage of final condensation by baking in order to impart to the filament the greatest elasticity and resistance to chemical reagents and solutions.

40 In accordance with a modification of our invention an alkyd resin (with or without plasticizing agents) may be spun from a solution into a coagulating bath in accordance with known practice in the artificial silk manufacture. With this end in view the alkyd 45 resin, while still in the A-stage is dissolved in solvents as for example in a mixture of acetone and alcohol and is extruded in filamentary form into a water bath or other coagulating agent, which may be at room temperature.

On leaving the coagulating agent the extruded material is dried and converted by baking to its C-stage, in which the resin is insoluble and non-fusible.

What we claim as new and desire to secure 55 by Letters Patent of the United States is:

1. An artificial silk consisting of a condensation product of polyhydric alcohol and polybasic acid.

2. A textile fibre consisting of a condensation product of glycerine and phthalic anhydride.

3. A textile fibre consisting of an alkyd resin in an insoluble, non-fusible condition.

4. A textile fibre consisting of a plasticized condensation product of polyhydric alcohol and polybasic acid.

In witness whereof, we have hereunto set our hands this 17th day of November, 1928.

HANS SCHUHMANN. 70  
FRIEDRICH STREUBER.

75

80

85

90

95

100